# EUROPEAN PATENT APPLICATION

(11) **EP 0 885 985 A1**
(43) Date of publication of application: **23.12.1998**
(21) Application number: 98201206.4
(22) Date of filing: 15.04.1998
(51) Int. Cl.: C23G 1/08, C23G 1/02, C23F 1/16

(54) **Method of treating a metal**

(30) Priority: 05.05.1997 EP 97850075
(71) Applicant: AKZO NOBEL N.V., 6800 SB Arnhem (NL); Eka Chemicals AB, 445 80 Bohus (SE)
(72) Inventor: Berglind, Troy, 423 54 Torslanda (SE); Frestad, Arne, 416 72 Göteborg (SE)
(74) Representative: Jönsson, Christer

(57) **Abstract**

The invention relates to a method of pickling or surface treating a metal in an aqueous solution containing nitric acid wherein hydrogen peroxide is supplied to decrease the formation of nitrous fumes. At least a portion of the hydrogen peroxide is supplied by spraying or flushing an aqueous solution thereof directly on the metal through one or several separate nozzles (18a, 18b, 19a, 19b).

## Description

The present invention relates to a method of pickling or surface treating a metal in a solution containing nitric acid to which hydrogen peroxide is supplied to decrease the formation of nitrous fumes.

At manufacturing of many metals such as steel, particularly stainless steel, an oxide layer forms at the surface during the annealing, and this layer must be removed. This is normally done by picking which means that the steel is treated in an acidic oxidising picking bath to affect some dissolution of metal under the oxide layer which then comes loose. Picking and surface treatment of metals is often performed in a solution based on nitric acid as an oxidising agent which treatment, however, involves emissions of nitrous fumes, mainly NO and NO₂. These emissions can be reduced significantly by adding hydrogen peroxide to the nitric acid containing solution as disclosed in the US patent 4938838 and 3945865 as well as in H. T. Karlsson et al, "Control of NOₓ in Steel Pickling", Environmental Progress, Vol. 3, No. 1, 1984, pp. 40-43. In picking of steel the following reactions occur: ${\text{2 Fe + 6 H}}^{\text{+}} {\text{+ 3 NO}}_{\text{3}} {\text{}}^{\text{-}} {\text{⇄ 2 Fe}}^{\text{3+}} {\text{+ 3 NO}}_{\text{2}} {\text{}}^{\text{-}} {\text{+ 3 H}}_{\text{2}} \text{O}$${\text{2 NO}}_{\text{2}} {\text{}}^{\text{-}} {\text{+ 2 H}}^{\text{+}} {\text{⇄ NO + NO}}_{\text{2}} {\text{+ H}}_{\text{2}} \text{O}$${\text{NO}}_{\text{2}} {\text{}}^{\text{-}} {\text{+ H}}_{\text{2}} {\text{O}}_{\text{2}} {\text{⇄ NO}}_{\text{3}} {\text{}}^{\text{-}} {\text{+ H}}_{\text{2}} \text{O}$

This process generally works very well, but it has been found that in order to decrease the emissions below a certain level far more than stochiometric amounts of hydrogen peroxide must be supplied. At the same time, increasing consciousness of environmental problems call for more effective reduction of nitrous fumes.

The present invention intends to solve the problem of further reducing the emissions of nitrous fumes or NOₓ, particularly NO and NO₂, without increasing the hydrogen peroxide consumption to unacceptable levels. According to the invention it has surprisingly been found that the reduction of NOₓ emissions can be improved considerably without significantly increasing the hydrogen peroxide consumption if at least a part of the hydrogen peroxide is sprayed or flushed directly on the metal instead of being added to the nitric acid containing solution, either directly into a tub in which the metal is treated or into a circulation conduit for the nitric acid containing solution.

Thus, the present invention concerns a method of picking or surface treating a metal in an aqueous solution containing nitric acid wherein hydrogen peroxide is supplied to decrease the formation of nitrous fumes. At least a portion of the hydrogen peroxide is supplied by spraying or flushing an aqueous solution thereof directly on the metal through one or several separate nozzles. Preferably the hydrogen peroxide is sprayed in a way to obtain as small droplets as possible which makes the reaction with the NOₓ more efficient. Although it is possible to supply substantially all the hydrogen peroxide through the separate nozzles, the preferred portion is from about 20 to about 80%, most preferably from about 40 to about 60% of the total amount of hydrogen peroxide supplied.

Without being bound to any theory it is assumed that hydrogen peroxide coming into contact with metal ions in a pickling solution decomposes catalytically into water and oxygen and is thus consumed to no use. It is also assumed that the main part of the nitrous fumes are generated at the surface of the metal and that the hydrogen peroxide therefore is most likely to contact the NOₓ before it comes into contact with metal ions if it is sprayed or flushed directly on the metal. This is supposed to be particularly true when nitric acid containing solution is sprayed or flushed directly on the metal in which processes considerable amounts of nitrous fumes evolve even at very low concentrations of dissolved NOₓ.

The nitric acid solution normally contains from about 0.1 to about 4 mols/l, preferably from about 0.5 to about 3 mols/l of nitric acid, and suitable also hydrofluoric acid, for example from about 0.01 to about 5 mols/l, preferably from about 0.1 to about 3 mols/l. The content of dissolved NOₓ is normally from about 0.01 to about 0.7 g/l, preferably from about 0.1 to about 0.4 g/l. The invention is particularly advantageous when the content of dissolved NOₓ is below about 0.7 g/l. Normally most of the dissolved NOₓ is in the form of NO₂⁻.

According to the invention it is generally possible to maintain the emissions of NOₓ gas below about 7 g NOₓ per m² treated metal and often even below about 4 g NOₓ per m² treated metal at a hydrogen peroxide consumption from about 2 to about 60 g H₂O₂, preferably from about 5 to about 40 g H₂O₂ per m² treated metal.

The amount of hydrogen peroxide added can be controlled by conventional method such a by measuring the redox potential in the nitric acid containing solution or measuring the content of NOₓ in the exhaust gas. Preferred redox potential control methods are described in US 4938838 and EP 442250.

The invention is advantageous in all processes for surface treatments of metals such as steel, copper or brass with nitric acid containing solutions. It is particularly advantageous in pickling of steel, especially stainless steel.

The invention will now be described in connection with the enclosed Figure schematically showing an embodiment of a process of treating a metal.

The figure shows a tub 1 containing a surface treating or pickling bath 2 of an aqueous solution containing nitric acid and preferably also hydrofluoric acid through which a running strip 3 of a metal, preferably stainless steel, is conducted continuously. Nitric acid containing solution is supplied through lances 5a, 5b, 6a, 6b, each containing a plurality of nozzles 7a, 7b, 8a, 8b spraying the solution on each side of the metal strip 3 so it is distributed over substantially the entire width thereof. Solution from the bath 2 is withdrawn to a tank 4 and is fed to the lances 5a, 5b, 6a, 6b at sufficiently high pressure via a circulation conduit 10 and a pump 11. The process also involves supply of an aqueous solution of hydrogen peroxide from at storage tank 12. A portion of the hydrogen peroxide is brought by a pump 13a to separate lances 16a, 16b, 17a, 17b, each containing a plurality of nozzles 18a, 18b, 19a, 19b spraying the solution on each side of the metal strip 3 so it is distributed over substantially the entire width thereof. The suitable number of nozzles depends on the size of the metal strip 3 and on the type of nozzles, but normally from about 4 to about 12 nozzles per lance is sufficient. Any conventional nozzle can be used, for example nozzles also blowing air which prevents clogging at interruption of the hydrogen peroxide flow. The remaining part of the hydrogen peroxide supplied is added by pumps 13b, 13c to the nitric acid containing solution in the tank 4 and the circulation conduit 10 at the suction side of the pump 11. The hydrogen peroxide from the pump 13c is preferably mixed with the solution from the bath 2 just before it enters the tank 4. Above the tub 1 a hood 25 containing a vent 26 is arranged. Any nitrous fumes formed is evacuated through the vent 26. The supply of hydrogen peroxide is preferably controlled on basis of the NOₓ content in the gas stream in the vent 26 or of the redox potential in the bath 2. It is also possible to have fixed flow of hydrogen peroxide added through the nozzles 18a, 18b, 19a, 19b and only regulate the pumps 13b, 13c supplying hydrogen peroxide to the tank 4 and the circulation conduit 10.

Although not shown in the Figure it is possible to treat the metal strip 3 without immersing it into the bath 2. It is also possible to convey the metal strip 3 vertically and spray the nitric acid containing solution and the hydrogen peroxide on the vertical surfaces.

The invention is further illustrated through the following example. If not otherwise stated all contents and percentages refer to wt%.

EXAMPLE: In a plant according to the Figure stainless steel was pickled in a an aqueous solution of 2.9 mols/l nitric acid and 2.7 mols/l hydrofluoric acid. When all the hydrogen peroxide was added to the nitric acid containing solution in the tank 4 and the circulation conduit a hydrogen peroxide consumption of 60-70 ml 35% aqueous H₂O₂ per m² pickled steel was required to keep a NOₓ concentration below 280 ppm in the vent 26 (corresponding to 3.5 g NOₓ per m² pickled steel). When the process was operated according to the invention and about 45% of the hydrogen peroxide supplied was sprayed directly on the steel surface through the separate lances 16b, 17b above the steel strip 3, each containing six nozzles 18b, 19b, the consumption required to keep a NOₓ concentration below 280 ppm in the vent 26 was only 40-45 ml 35% aqueous H₂O₂ per m² pickled steel.

## Claims

1. A method of pickling or surface treating a metal in an aqueous solution containing nitric acid wherein hydrogen peroxide is supplied to decrease the formation of nitrous fumes **characterised** in that at least a portion of the hydrogen peroxide is supplied by spraying or flushing an aqueous solution thereof directly on the metal through one or several separate nozzles (18a, 18b, 19a, 19b).

2. A method as claimed in claim 1, **characterised** in that from about 20 to about 80% of the total amount of hydrogen peroxide supplied is supplied through the separate nozzles (18a, 18b, 19a, 19b).

3. A method as claimed in claim 2, **characterised** in that from about 40 to about 60% of the total amount of hydrogen peroxide supplied is supplied through the separate nozzles (18a, 18b, 19a, 19b).

4. A method as claimed in any one of the claims 1-3, **characterised** in that from about 2 to about 60 g H₂O₂ per m² treated metal is supplied.

5. A method as claimed in any one of the claims 1-4, **characterised** in that nitric acid containing solution is sprayed directly on the metal.

6. A method as claimed in any one of the claims 1-5, **characterised** in that the nitric acid solution contains from about 0.1 to about 4 mols/l of nitric acid.

7. A method as claimed in any one of the claims 1-6, **characterised** in that the content of dissolved NOₓ in the nitric acid containing solution is below about 0.7 g/l.

8. A method as claimed in any one of the claims 1-7, **characterised** in that the metal is steel.

9. A method as claimed in any one of the claims 1-8, **characterised** in that the emissions of NOₓ is maintained below about 7 g per m² pickled metal.

10. A method as claimed in any one of the claims 1-9, **characterised** in that the nitric acid containing solution also contains hydrofluoric acid.
